

## UNITED STATES PATENT OFFICE.

ADOLF BECK, OF GRIESHEIM-ON-THE-MAIN, GERMANY, ASSIGNOR TO CHEMISCHE  
FABRIK GRIESHEIM-ELEKTRON, OF GRIESHEIM-ON-THE-MAIN, GERMANY.

## CASTING METALS.

No Drawing.

Application filed July 16, 1923. Serial No. 651,959.

My invention refers to the melting and casting of easily oxidizable metals such as magnesium and its alloys. It is an object of my invention to provide means whereby 5 the oxidizing action of steam on castings of such metals is prevented, especially as regards castings made in sand moulds.

As is well known to those skilled in the art, if it is intended to cast metals, such as 10 magnesium and its alloys, which are liable to get oxidized in heated condition, the casting being effected with the aid of the sand moulds hitherto generally employed, such moulds must be carefully dried, in order to 15 obtain good castings. If the moulds are not dried carefully, a reaction will take place between the metal and the water present in the mould and more especially in the sand, and a similar reaction is then liable to take 20 place between the metal and the moulding material, such as sand, such reaction rendering the casting at least inferior in outer appearance. If great quantities of water are 25 still present in the mould, explosion-like phenomena are even likely to occur.

In an application for patent of the United States Ser. No. 563,717, filed on May 25, 1922 by Karl Gersbach, Oskar Hermann Weber and myself a method of casting is 30 described which allows avoiding the ignition of the metal, provided that the moulds are carefully dried, this method substantially consisting in providing the mould with a coating of a material which will not 35 react with the molten metal, either as such or in the form of its products of oxidation. I assume this protective effect to be due to the action of the gases or vapors developed from the protective material in contact with 40 the hot metal and which prevent the access of air or steam to the metal.

I have now ascertained that by employing certain materials in the preparation of the mould for casting, I obtain the surprising 45 result that the drying of the mould and of the sand contained therein is no more necessary, the presence of water being innocuous so that I am now enabled to cast the metals in question in comparatively wet moulds. These materials (which may be 50 called protective substances) are those described in the specification above cited, as being adapted to prevent oxidation of the castings when intensely dried moulding sand 55 is used, and more especially sulphur and

compounds of oxalic acid. Moreover, I have found that bicarbonates, urea, boric acid, as well as mixtures of these substances have proved suitable. The peculiar action of the protective substance has not yet been cleared 60 up completely. It seems that the steam and air are sufficiently diluted with gases or vapors produced from these substances or that they prevent in some other way the access of water vapor to the hot metal so 65 that no visible action of the steam upon the metal occurs. However, I wish it to be understood that this is merely an attempt to explain the peculiar action of the protective substances. 70

I may apply the protective materials in the form of a watery paste, suspension or emulsion on the surface of the mould after it has set, or I may admix a suitable quantity of such materials to the sand before making 75 the mould.

If sulphur is employed as protective material and sand as moulding material, an addition of 1-6% sulphur to the sand has proved advantageous. I prefer admixing 80 the protective material to the sand or the like for the reason that the powdering or spraying on will sometimes be difficult in such places of the mould which are not easily accessible. Moreover, by admixing the protective material to the sand a sound protective 85 effect is obtained even at those places where the casting is comparatively thick such as gates, inasmuch as the protective gases or vapors are not developed merely on the surface of the mould, as in the case of superficial powdering or spraying on, but also from deeper layers in correspondence with the gradual heating of the mould by the metal 90 as it flows in. However, in certain cases I 95 may admix the protective material to the sand and besides powder or spray it onto the mould.

If boric acid is employed as protective material instead of sulphur, an addition of 100 0.2-1 per cent to the sand has proved sufficient.

A similar effect within the scope of my invention might be obtained also by developing gases or vapors from the protective materials spoken of above out-side the mould and introducing them into the mould immediately before the casting. However, if this is done, the protective effect will be less 105 powerful for the reason that the concentra- 110

tion of the protective masses or vapors will not be as great between the mould and the metal, as if they are generated in the mould itself.

5 I wish it to be understood that I do not desire to be limited to the particular substances and modes of proceeding described, for obvious modifications will occur to a person skilled in the art.

10 I claim:

1. The method of preventing easily oxidizable metals and alloys for oxidizing on being cast in undried moulds, comprising mixing moulding material with a non-metallic substance incapable of reaction with said metal and adapted, when heated by the heat emitted from the cast metal, to form on the surface of the casting a layer preventing the casting being spoilt by the access of air and water vapor.

15 2. The method of preventing easily oxidizable metals and alloys for oxidizing on being cast in undried moulds, comprising

mixing moulding material with a non-metallic substance incapable of reaction with 25 said metal and adapted, when heated by the heat emitted from the cast metal, to form on the surface of the casting a layer preventing the casting being spoilt by the access of air and water vapor, forming said mixture into 30 a mould and covering the surface of said mould with said substance.

3. The method of preventing easily oxidizable metals and alloys for oxidizing on being cast in undried moulds, comprising 35 mixing with the moulding material boric acid.

4. The method of preventing easily oxidizable metals and alloys for oxidizing on being cast in undried moulds, comprising 40 mixing with the moulding material a quantity of boric acid substantially not exceeding 1 per cent of such material.

In testimony whereof I affix my signature.

ADOLF BECK.